

Feb. 1, 1949.

R. H. K. THOMSON

2,460,372

MANUFACTURE OF ARTIFICIAL PROTEIN FILAMENTS

Filed Aug. 21, 1944



Inventor  
ROBIN H. K. THOMSON

Cushman, Darby & Cushman

Attorneys

## UNITED STATES PATENT OFFICE

2,460,372

## MANUFACTURE OF ARTIFICIAL PROTEIN FILAMENTS

Robin H. K. Thomson, Kilwinning, Scotland, assignor to Imperial Chemical Industries Limited, a corporation of Great Britain

Application August 21, 1944, Serial No. 550,487  
In Great Britain October 20, 1943

12 Claims. (Cl. 18—54)

1

The present invention relates to the manufacture of filaments of coagulated and insolubilised protein material for textile purposes, and more particularly to a process for the improvement of filaments obtained by a wet spinning process from solutions of casein or vegetable globulins, which have been subjected in coagulated filamentary form to the action of an acidified aqueous solution of formaldehyde or other aqueous insolubilising bath adapted to render the coagulated protein filament capable of withstanding hot weakly acid or alkaline solutions such as are used in dyeing and laundering.

In the production of insolubilised wet spun protein filaments it is usual to apply a stretch to the filament at some part of the process, and to effect at least a partial stabilisation of the length of the stretched filament by means of the baths through which it passes; so that when the tension is released it will not shrink excessively in a longitudinal direction. This stretching and length stabilisation may be effected prior to the commencement of the insolubilisation, or in the course of the insolubilisation of the coagulated protein. In either case the insolubilised filaments obtained after the release of any tension upon them are substantially unstrained and exhibit little or no bi-refringency.

It is known that textile filaments of various kinds can be improved in strength by steaming them in stretched condition and drying them off while still stretched, but the improvement so obtained is usually lost when the filaments are subsequently subjected in the untensioned condition to the action of boiling water or steam.

We have now found that when insolubilised, crimped or uncrimped, protein filaments are wet stretched and are subsequently subjected to the action of formaldehyde for a period of time, and set by drying them at high temperature, both of these operations being conducted while they are held stretched, they become markedly bi-refringent and their untensioned length and strength are increased, and the longitudinal shrinkage and loss of strength when the resulting filaments are subsequently treated for example with boiling water in the untensioned condition is less than when the formaldehyde treatment is omitted, but is sufficient to give them a crimp.

According to the present invention, therefore, the process for the production of improved and crimped filaments from insolubilised filaments obtained by wet-spinning from solutions of casein or vegetable globulins comprises wet-stretching

2

the said insolubilised filaments, retaining the filaments in the stretched condition while subjecting them to raised temperature and treatment with formaldehyde, and thereafter withdrawing the tension and effecting the shrinkage of the thus treated filaments to the desired degree of crimp.

If desired the wet stretched filaments may be dried off under tension at raised temperature before the formaldehyde treatment is commenced. The drying is conducted at a temperature not less than 80° C., and if desired the filaments may be further heated to a temperature of 100° to 120° C. before commencing the formaldehyde treatment.

15 The wet stretching is advantageously carried out with hot water or steam, and the extent to which the insolubilised filaments can be stretched without breaking, may depend on the nature of the treatment they have received in their production, but it will usually be possible to apply a

stretch of from 50 to 100 per cent. The stretched and if desired dried filaments may then be immersed in commercial formalin solution, i. e. a solution of formaldehyde of a lower acidity

20 than that used in the previous insolubilisation step and left in contact with the solution for several hours if it is used at ordinary temperature. However, instead of immersing the filaments in a formaldehyde solution they can be subjected

25 to an atmosphere of formaldehyde vapour. The formaldehyde treated filaments may then be washed until their odour is faint and are then dried at a raised temperature not below about 80° C. Preferably the temperature is allowed

30 to rise somewhat about 100° C. when they have been dried. The tension on the filaments may then be released. At this stage they are straight and silk-like, but on immersion in hot water they shrink, and after drying in untensioned condition have a desirable woolly crimp.

In putting the invention into effect it is convenient to carry out the wet stretching of the insolubilised filament, and the subsequent steps in which it is maintained in stretched condition,

45 with a continuous length of filament, which implies that the whole of the preceding steps in the production of filaments, including the insolubilisation treatment, is also carried out before cutting the filaments.

50 It is desirable to wash the insolubilised filaments at least substantially free from the insolubilising solution before the wet stretching step is carried out. Before the wet stretching step is carried out it is permissible to relieve the insolubilised filaments of any tension under which they

are held, and frequently it is desirable to do so. If the continuity of the operations is thus broken, the insolubilised and washed filaments may be dried off and stored for any convenient period before the treatment according to the present invention is commenced. On the other hand, it is not essential that there should be any such break in the continuity, for the washed insolubilised filaments, whether or not already under tension, may be directly subjected to the wet stretching step.

A more complete understanding of the procedures of this invention may be had by reference to the accompanying drawing which diagrammatically illustrates the procedural steps involved. In the drawing,

Figure 1 shows the three preliminary stages of spinning, insolubilizing and washing of the filaments;

Figure 2 shows the subsequent steps of drying and hot drawing of the filaments;

Figure 3 illustrates the steps of treating the filaments while under tension to insolubilizing, washing and hot drying steps, and

Figure 4 shows the steps of rewinding the tensioned filaments into hank form and subsequently treating the untensioned filaments to boiling and drying.

Referring in detail to the drawings, the filament 2 is formed by extruding a protein solution through the spinneret 4 into the coagulated bath 6 and thence to the hanking device where hanks 8 are formed. The hanks are then placed in the insolubilizing bath 10, where the filaments are insolubilized, after which they are passed into a washing bath 12. Since the drawing is only diagrammatic in nature, only one washing tank is illustrated but it will be understood that several such tanks may be employed and that pure water or weak alkaline or other washing solutions may be employed.

From the washing tank, the filaments are passed to a hot air drier 14 where the filaments are and subjected to the drying action of hot air. Thence, the dried filaments are passed from winding the roll 16 to tension rollers 18 and 20 through the steam chamber 24 and are wound upon the winding roller 26 at a speed in excess of the speed of the tension rollers 18 and 20, so that the filaments are elongated while within the steam chamber 24 and subjected to the action of the steam passed through this chamber.

The filaments are retained under the tension produced during the winding operation upon the rollers or bobbins 28. In this condition, they are first immersed in an insolubilizing bath 30 from where they are taken and immersed in the washing bath 32. Finally, while still under tension, the filaments are dried in the drying chamber 34 by hot air.

The bobbin of tensioned filament 28 is then rewound onto a roller 36 so that the filaments may be formed in hanks for further treatment in an untensioned condition. In the untensioned state, the filaments are immersed in the boiling water tank 38. Finally, the filament hanks are dried in the hot air drying chamber 40.

The invention is illustrated by the following example:

#### Example

The filaments employed as the starting material are prepared by coagulating in a hot acidified sodium sulphate bath under tension a viscous aged solution of peanut protein in dilute

aqueous sodium hydroxide solution, the protein solution being extruded into the coagulating bath through a multiple hole spinneret, and subsequently insolubilising the coagulated filaments in the untensioned condition in a bath consisting of a nearly saturated solution of sodium chloride containing 1 per cent formaldehyde and 1.75 per cent sulphuric acid for a period of 18 hours at 20° C., and then washing the filaments, treating them first, with an aqueous dispersion of "Lissapol C," then with a dilute sodium carbonate solution, and then drying them off in hank form. The use of the hot coagulating bath effects a sufficient stabilisation of their length to enable the insolubilisation treatment with the acidified saline formaldehyde solution to be carried out in the untensioned condition. The treatment with the "Lissapol" dispersion confers a somewhat softer handle on the filaments, and the treatment with dilute sodium carbonate solution is intended to raise the pH of the filaments to a value of about 7, which is frequently desirable for dyeing purposes. The drying of the filaments is carried out in hot air at 100° C. The resulting filaments have a considerable crimp, and exhibit little birefringence. Their tensile strength is approximately 8 kilograms per square millimetre, as calculated on their average thickness from the breaking stress in an atmosphere of 50 per cent. relative humidity at 20° C.

The dried filaments are then thoroughly damped in steam and the filaments are drawn off from it through the steam to a roller on which they are wound helically under such tension that their taut length is increased about 75 per cent. The rollers carrying the filaments in the stretched state are then immersed for 16 hours in commercial formalin solution.

The filaments are then washed until substantially free from odour and dried in air at 100° C. under tension, and are then released from the tension. The resulting filaments have no crimp and have an artificial silk-like appearance. They are relatively strongly bi-refringent. Their tensile strength is approximately 12 kilograms per square millimetre, as calculated in the manner already referred to. The resulting filaments are now rewound into hank form and are immersed in boiling water in the untensioned condition for 10 minutes. They are then dried off in air at 100° C. without tension; as a result of this treatment they acquire a useful degree of crimp and a wool-like appearance. They are then rehumidified. Their tensile strength is approximately 9.7 kilograms per square millimetre, as calculated in the manner already referred to. They are intermediate in bi-refringency between the insolubilised filaments employed as the starting material and the artificial silk-like filaments already referred to.

I claim:

1. The process for obtaining an improved, crimped, protein filament, which comprises wet-stretching an insolubilized filament previously formed by wet-spinning a protein solution of the group consisting of vegetable globulin solutions and casein solutions, contacting the taut filament with formaldehyde, drying the taut filament at a temperature of at least 30° C., releasing the tension on the filament and thereafter contacting the filament in relaxed condition with boiling water.

2. The process for obtaining an improved, crimped, protein filament, which comprises stretching in steam an insolubilized filament

## 5

previously formed by wet-spinning a vegetable globulin solution, contacting the taut filament with formaldehyde, drying the taut filament at a temperature of at least 80° C., releasing the tension on the filament and thereafter immersing the filament in relaxed condition in boiling water.

3. The process for obtaining an improved, crimped, protein filament which comprises stretching in steam a formaldehyde-insolubilized filament previously formed by wet-spinning a vegetable globulin solution, drying the taut filament at a temperature within the range of from 80° C. to 120° C., immersing the taut filament in an aqueous formaldehyde solution, washing the taut filament, drying the taut filament at a temperature of at least 80° C., releasing the tension on the filament and thereafter immersing the filament in relaxed condition in boiling water.

4. The process for obtaining an improved, crimped, protein filament, which comprises stretching in steam a washed, formaldehyde-insolubilized filament previously formed by wet-spinning a sodium hydroxide peanut protein solution, drying the taut filament at a temperature within the range of from 100° C. to 120° C., immersing the taut filament in a formalin solution, washing the taut filament, drying the taut filament at a temperature of at least 100° C., releasing the tension on the filament and thereafter immersing the filament in relaxed condition in boiling water.

5. A crimped protein filament formed according to the process set forth in claim 1.

6. A crimped protein filament formed according to the process set forth in claim 3.

7. A process for producing crimped, protein filaments of relatively high tensile strength which comprises wet-spinning a protein solution into a coagulating medium, insolubilizing the resulting filaments in an acidic saline formaldehyde solution, stretching while wet the insolubilized filaments, contacting the taut filaments with formaldehyde, drying the resulting taut filament at a temperature between 80° C. and 120° C., releasing the tension on the filaments and, thereafter, immersing the filament in a relaxed condition in boiling water.

8. A crimped protein filament formed according to the process set forth in claim 7.

9. A process for producing crimped, peanut protein filaments of relatively high tensile strength which comprises wet-spinning a solution of peanut protein dissolved in an aqueous sodium hydroxide solution into a coagulating medium, insolubilizing the resulting filaments in an acidic

## 6

saline formaldehyde solution, stretching while wet the insolubilized filaments to between a 50 and 100% increase in length, immersing the taut filaments in an aqueous formaldehyde solution, drying the resulting taut filament at a temperature between 80° C. and 120° C., releasing the tension on the filaments and, thereafter, immersing the filament in a relaxed condition in boiling water.

10. A process for producing crimped, peanut protein filaments of relatively high tensile strength which comprises wet-spinning a solution of peanut protein dissolved in an aqueous sodium hydroxide solution into a coagulating medium, treating the resulting filaments in an acidic saline formaldehyde solution for a sufficient length of time to make the filaments completely resistant to the action of boiling water and hot dilute acid, stretching the insolubilized filaments in steam, immersing the taut filaments in an aqueous formaldehyde solution, drying the resulting taut filament at a temperature between 80° and 120° C., releasing the tension on the filaments and, thereafter, immersing the filament in a relaxed condition in boiling water.

11. The process of claim 10 wherein said treatment with acid saline formaldehyde is carried out on the filaments for about 18 hours at 20° C.

12. The process of claim 11 wherein the immersion of the taut filaments in the formaldehyde solution is carried out for about 16 hours at 20° C.

ROBIN H. K. THOMSON.

## REFERENCES CITED

The following references are of record in the file of this patent:

## UNITED STATES PATENTS

| Number    | Name          | Date           |
|-----------|---------------|----------------|
| 379,672   | DeKadt        | Apr. 27, 1943  |
| 2,211,961 | Meigs         | Aug. 20, 1940  |
| 2,290,789 | Wormell       | July 21, 1942  |
| 2,293,989 | Lely          | Aug. 25, 1942  |
| 2,338,916 | Ferretti      | Jan. 11, 1944  |
| 2,340,909 | Traill et al. | Feb. 8, 1944   |
| 2,358,427 | Traill        | Sept. 19, 1944 |

## FOREIGN PATENTS

| Number  | Country       | Date          |
|---------|---------------|---------------|
| 502,710 | Great Britain | Mar. 23, 1939 |

## OTHER REFERENCES

I. and E. Chem., December 1940, pages 1547-551. (Copy in Div. 15.)